

## UNITED STATES PATENT OFFICE

2,159,588

PROCESS FOR THE PHOTOMECHANICAL  
MANUFACTURE OF PRINTING FORMS FOR  
INTAGLIO PRINTINGJosef Görig, Loevenich, near Cologne, Germany,  
assignor to firm Bekk & Kaulen Chemische  
Fabrik G. m. b. H., Loevenich, near Cologne,  
GermanyNo Drawing. Application March 4, 1936, Serial  
No. 67,068. In Germany April 2, 1935

10 Claims. (Cl. 95—5.7)

The usual procedure for the manufacture of printing forms for intaglio copperplate printing and the like working with a doctor consists in first copying the image to be reproduced on a light-sensitive carbon tissue, whereupon the produced copy is transferred by dabbing to the printing form and is treated and etched here in the customary way. But the use of the carbon tissue for the manufacture of deeply etched printing forms has the disadvantage, that this paper is very sensitive against atmospheric influences, and this is most unfavourable especially in the manufacture of polycolour reproductions. Since the carbon tissue changes most easily its shape and especially its size under the influence of weathering, there is always danger that the transferred image proves to be larger for one colour than for another. Under such circumstances, however, some etching or other will easily become unsuitable, particularly for quality work. It is from this reason that till now by intaglio copperplate printing generally only reproductions in one colour were manufactured. Coloured reproductions are mostly printed only on small machines one up, so that the whole printing cylinder may be slided and rocked till the mono-coloured images will fit correctly on one another. But when larger sizes are used, it is not possible to handle the printing cylinder in such a manner, that the single impressions or images may be brought to fit on one another exactly.

This drawback is eliminated by the procedure according to the present invention. For this purpose no carbon tissue at all is used here, but the metallic support utilised for the printing form (plate, cylinder or the like) is coated with a colloid layer rendered light sensitive, and the image is then copied directly on this light sensitive layer, and the latter is screened to produce the edges supporting the doctor. The screen may be copied upon the light sensitive layer, as desired, before or after the image is copied, by means of a diapositive. In such cases where the printing form shall be used at the same time for the reproduction of characters, the latter and the image may be mounted jointly on one glass plate, so that characters and image may be copied at the same time upon the light sensi-

tive layer of the printing form. When image and screen are transferred to the base of the printing form by exposure to light, the treatment with an etching solution is performed in accordance to the present invention. Preferably such etching solutions are used, which, besides the usual mordant, like ferric chloride, contain an acid of such a kind, as for instance lactic acid or the like, which attacks or penetrates and swells the not hardened colloid layer but does not corrode or attack the metal of the plate or the like. There is no need in this case to coat with bituminous varnish the places not to be etched, since the hardened parts of the colloid layer are thoroughly proof against the mordant.

It further has been proved, that not rarely difficulties are met in obtaining useful prints from the printing forms produced by the present method, and that these difficulties are due to an insufficient or defective formation of the edges for supporting the doctor. It has been found that the imperfect formation of these edges was caused here by insufficient hardening of the light sensitive layer during the copying of the screen.

This is a surprising statement, because such difficulties are not met when the pigment paper process is used. When applying equal and equally thick and equally sensitised colloidal layers on the one hand for the carbon tissue according to the known process, and on the other hand for the metallic body of the printing form according to the present method, the very time and degree of exposure which is thoroughly sufficient to produce the edges for supporting the doctor in the former case, frequently does not suffice to accomplish with certainty those edges on the printing form in the process of the present invention.

This observation may be accounted for in the following manner: When working with carbon tissue those parts of the light sensitive layer which originally were on the top side of the paper lie underneath, i. e. in direct touch with the metallic support when the sensitive layer is dabbed to the latter. Now as at the surface of the layer the hardening is naturally greatest when the sensitive layer is exposed in order to copy the screen, there is full security that the strongest hardened parts of the layer are

brought into immediate contact with the metallic support of the printing form when said layer is dabbed on the metal. Consequently one can be sure that on developing and etching the screen copy to produce the edges for supporting the doctor or the like, these edges will perfectly appear on the metallic printing form, no matter whether the exposure has been a short or a longer one.

10 But things are different, if according to the present invention the half tone image and the screen are transferred directly to a light sensitive layer which has previously been arranged on the metallic support. For in this case that 15 part of the layer which by exposure is hardened most lies on the top, whereas the least hardened part lies on the underside, i. e. in contact with the metallic support. Now, if the exposure in copying the screen is not long enough, it may 20 happen that in developing and etching the light sensitive layer, the developing and etching means intrude laterally through the non-exposed parts of the surface beneath the superficially hardened parts of the edges produced 25 by copying the screen. Then the latter are removed when the parts of the layer which have remained unexposed are dissolved or removed, and thus the edges for supporting the doctor will no more be formed in a satisfactory manner 30 when the metal form is etched.

Accordingly, when the screen is copied on the sensitive layer of the metal form it is important for the process of the present invention to expose during such a time that there will be perfect security, that the exposed spots of the sensitive layer are thoroughly hardened down to the basis, i. e. to the surface of the metal form. If the exposure has been so lengthened in this 35 way, the same reliability will exist here for the completion of the edges as with the pigment paper process, and therefore perfect prints then are to be obtained here also with certainty.

It may easily be ascertained, if needed by a preliminary test, what time of exposure will be 40 required to attain the desired aim in any particular case. By using a given source of light and a sensitive layer of definite composition and sensitisation, and of given thickness one may 45 ascertain what time is wanted in order to arrive at a perfect completion of the edges for supporting the doctor on the metallic support by etching, if the screen is copied alone, i. e. without the half tone image. In this direction experience has shown what follows:

50 With the pigment paper process the time for copying the screen should be longer by about one quarter of the time required for copying the half tone image, say for instance 8 minutes for the screen against 6 minutes for the half tone image. Now, all other things being equal, it 55 has proved suitable, when using the process of the present invention, to expose for the copying of the screen about thrice as long as for the copying of the half tone image, say for instance 60 about 18 minutes against 6 minutes.

The process according to the present invention may be executed in different ways and manners. The layer of the light sensitive colloid may consist of a chromatised glue soluble in 65 warm water, like the chromatised so-called "Beka" photoengraving glue (as manufactured by Messrs. Dr. Bekk & Kaulen Chemische Fabrik G. m. b. H., of Loevenich, near Cologne), or chromatised gum arabic. After the screen and 70 the diapositive or the like are copied on this

layer by exposing them, the one after the other, during the time required in accordance to what has been said above, the etching solution is brought on the plate or the like without previous development. Preferably the etching solution in 5 this case is composed in such a way, that is to say it shall suitably have such a viscosity, that the copying layer, even if not exposed to the light, would not be influenced by the ferric chloride solution as such, but that the added weak acid attacks and penetrates those parts of the colloid layer, which are not hardened at all or only to a relatively low degree. As an etching solution adapted for this purpose may be taken a ferric chloride solution of 48-50° Bé with an 10 addition of 3-5% lactic acid.

When those parts of the colloid layer which were not exposed at all or only in a relatively small measure are brought to swelling by the lactic acid, the ferric chloride can act at the 15 penetrated spots on the metal of the printing form, whereas the weak acid itself neither does nor need corrode the metal. The copying or colloid layer is brought to swelling by this acid of course in such a way that those image spots 20 which were exposed least are attacked first, and that the further swelling of the layer takes place gradually and by steps corresponding to the degree of hardening of the layer. The quantity of the acid added to the etching solution must be 25 chosen such that the edges for the doctor formed by the screen and hardened by the high exposure are not attacked by this acid.

Instead of lactic acid, other acids of similar efficiency may be applied, preferably organic 30 ones, which are suited to cause the nonhardened parts of the colloid layer to swell, but to leave unattacked the hardened parts and which do not attack at all or only to a small degree the metal 35 of the form.

After the treatment with the acidulated mor- 40 dant, if necessary, a treatment with an etching bath of the usual kind, for instance a ferric chloride solution of appropriate concentration, may take place. When the etching procedure is 45 finished, the printing form is freed from the hardened colloid layer left on the form, for instance by the aid of caustic alkalis, of weak sul- 50 furic acid (of about 1% content), or the like, and, after repolishing, it then will be ready for the 55 printing process in the machine.

For the manufacture of the printing form, instead of the chromatised glue or gum soluble 60 in warm water as mentioned above, a layer of chromatised gelatine may be employed which is 65 produced by means of the unchanged gelatine as it is on sale and which quickly sets and only swells in warm water without dissolving. In this case the image after having been transferred to the chromatised layer in an adequate man- 70 ner and after the latter having been screened by exposure may first be developed in water. The temperature of the developing water, how- 75 ever, then ought to be such, that the gelatine is not dissolved even at the spots not exposed to the light and consequently not hardened, but here is made only to swell. The water tempera- 80 ture to be used for the development, consequently, depends upon the quality of the gelatine used and may easily be found out by a previous test. 85 Generally, when using the gelatine of the trade (edible gelatine), for this reason a temperature of 40-45° C. should not be substantially exceeded. Since the gelatine is not dissolved by the water 90 performing the development, after the comple- 95

tion of the latter the gelatine will yet be present on the plate as an apparently uniform uninterrupted layer. During the subsequent etching those parts of the gelatine layer, which were unexposed or less exposed and made to swell by the development, are more readily penetrated by the mordant than the parts hardened more or less. This even then will be the case if only the normal mordants are used, such as ferric chloride solution without addition of any acid. In this case, therefore, only those normal mordants need be used. According to the less or greater degree of hardening of the respective spots the mordant will penetrate more quickly or more slowly through the gelatine layer to the metal and will effect here the correspondingly graduated etching. After etching the gelatine layer may be removed in a corresponding manner as in the procedure described before.

It has been found to be suitable in this second named form of execution of the new process to add a finely divided filler to the gelatine before the latter is spread over the metal plate or the like. By means of the filler on the one hand the rapid setting of the gelatine when spread by whirling or the like over the plate or the like may be delayed whereby the formation of a uniform layer is facilitated. On the other hand the deep etching may be favourably influenced thereby, as the filler will be washed out during the development preferably or only from those spots of the layer which are hardened not at all or only a little. As the degree of hardening and of swelling dependent thereupon may be, more or less of the filler will be washed out of a certain part of the gelatine layer. The latter, however, will be more readily penetrated by the etching means at the spots more freed from the filler than at those places, which retain still more or all of it. Thus the gradation of the tone in the etched image will be furthermore influenced favourably.

All such finely powdered substances are suitable as fillers for the aforesaid purpose, that can be uniformly divided in the gelatine and remain finely suspended during the spreading and drying of the latter on the metal plate, therefore not being settled too rapidly. Preferably as fillers pigments may be used, f. i. the red pigment of Messrs. H. Schmincke & Co., of Dusseldorf. The use of such pigments yet offers the particular advantage that at the same time a coloration of the gelatine layer is caused and therefore the inspection of the developed gelatine image is facilitated, as during the development more or less of the pigment is dissolved out of the parts of the layer hardened not or less. For instance a cleaned copper plate may be coated for this purpose in the whirler with a copying mixture composed of 1000 ccm. of water, 120 gr. of edible gelatine, 100 ccm. of "Beka" photoengraving glue, and 100 gr. of a red body-colour. This solution or mixture may be sensitised with equal parts of a 4% solution of potassium bichromate. The addition of the glue to the gelatine here also is intended to prevent too rapid a setting of the gelatine on the plate, and thus to facilitate the formation of a thoroughly uniform film or layer.

After the plate or the like is exposed under the diapositive or the like and under the screen during the required time, the development is carried out. For this purpose the plate is suitably first put into warm water where it is left, for instance, for about two minutes. Then it is brought into a dyeing and hardening bath, which for instance

may consist of 1000 ccm. of water, 20 to 30 gr. of water-soluble aniline dye, like methyl violet, and 40 to 50 gr. of alum. After some minutes the plate is taken out of this bath, and the development then is finished in warm water. The used water soluble aniline dye also serves the purpose to facilitate the examination of the developed image or of the degree of development reached, since during the final development in warm water this dye is washed out or away from those places where the unhardened swollen or relatively little hardened gelatine is to be found. It is self-explanatory that the dyeing with aniline dye, if desired, may be employed also where no filler like a pigment was added to the colloid solution. The tanning agent, f. i. alum, added to the middle bath confers to the layer the necessary stability during etching and contributes furthermore to promote the gradation of the latter according to the tone values of the image or picture. Instead of alum any other suitable tanning agent may be used, f. i. formaline or the like. There is no need to treat with the tanning means in the same bath as with the dyeing solution, but they may be effected independently from one another. Also, the treatment with the tanning agent, or with the dyeing solution, or with both agents may be omitted. On the other hand the tanning may be combined with the etching by adding the tanning means to the etching solution.

When the plate is developed and dried, in this form of execution all spots not to be etched are covered with varnish, and then the etching is performed in the otherwise usual way, for instance with ferric chloride solution of varying composition and concentration. In this case, of course, the etching may be performed under full daylight, in contrast to the first example of execution where the undeveloped image was to be etched. After the etching is finished, first the varnish is removed and then the remaining copying layer, if desired by means of water and emery powder or the like.

The process according to the present invention is suited in first line for the manufacture of planographic intaglio printing forms, but it may also be employed for the manufacture of rotary intaglio printing forms. As metal for the plates or the like, copper is the most important, but in certain cases other metals, such as brass, zinc or aluminum may also be employed.

Having now particularly described and ascertained the nature of my said invention, I declare that what I claim is:

1. A process for the photomechanical manufacture of printing forms for intaglio printing by means of a doctor which comprises covering a metallic body used as the basis for the printing form with a light sensitive chromatized colloid layer, exposing the same twice, under a diapositive of a continuous unscreened half-tone image and under a photogravure screen in any succession, the one after the other, and then treating said metallic body covered with the undeveloped, twice exposed colloid layer with a swelling means and an etching means.

2. A process for the photomechanical manufacture of printing forms for intaglio printing by means of a doctor which comprises covering a metallic body used as the basis for the printing form with a light sensitive chromatized colloid layer, exposing the same twice, under a diapositive of a continuous half-tone image and under a photogravure screen in any succession, the one after the other, the exposure for copying the

photogravure screen being made for a longer period than that independently made for copying the continuous half-tone image and for such a time, that those parts of the sensitive layer the surface of which is directly met by the light during the copying of the photogravure screen are hardened with certainty down to the base of said sensitive layer, and thereafter treating said metallic body with the undeveloped, twice exposed colloid layer with a swelling means and an etching means.

3. A process for the photomechanical manufacture of printing forms for intaglio printing by means of a doctor which comprises covering a metallic body used as the basis for the printing form with a layer of gelatine of the trade of such a kind which only will swell on being treated with warm water without dissolving and which is rendered light sensitive by chromatizing, exposing said sensitive layer twice, under a diapositive of a continuous half-tone image and under a photogravure screen in any succession, the one after the other, then treating said twice exposed gelatine layer with water of such a temperature, that the gelatine is not dissolved even at the unexposed spots but is only caused to swell at said spots, and thereafter subjecting said printing form to the action of an etching means.

4. A process for the photomechanical manufacture of printing forms for intaglio printing by means of a doctor which comprises covering a metallic body used as the basis for the printing form with a light sensitive chromatized colloid layer, exposing the same twice, under a diapositive of a continuous half-tone image and under a photogravure screen in any succession, the one after the other, and then treating said metallic body with the undeveloped, twice exposed colloid layer simultaneously with swelling-etching means, said means consisting of a mixture of an etching salt and a weak organic acid, said organic acid being capable to penetrate the unexposed, unhardened part of said colloid layer but not capable to attack said metallic body of the printing form.

5. A process for the photomechanical manufacture of printing forms for intaglio printing by means of a doctor which comprises covering a metallic body used as the basis for the printing form with a light sensitive chromatized colloid layer, exposing the same twice, under a diapositive of a continuous half-tone image and under a photogravure screen in any succession, the one after the other, and then treating said metallic body with the undeveloped, twice exposed colloid layer simultaneously with swelling-etching means, said means consisting of a mixture of an etching salt and lactic acid.

6. A process for the photomechanical manufacture of printing forms for intaglio printing by means of a doctor which comprises covering a metallic body used as the basis for the printing form with a light sensitive chromatized colloid layer, exposing the same twice, under a diapositive of a continuous half-tone image and under a photogravure screen in any succession, the one after the other, and then treating said metallic body with the undeveloped, twice exposed colloid layer simultaneously with swelling-etching means, said means consisting of a mixture of ferric chloride and lactic acid.

7. A process for the photomechanical manufacture of printing forms for intaglio printing by means of a doctor which comprises covering a metallic body used as the basis for the printing

form with a layer of gelatine of the trade of such a kind which only will swell on being treated with warm water without dissolving and which is rendered light sensitive by chromatizing, exposing said sensitive layer twice, under a diapositive of a continuous half-tone image and under a photogravure screen in any succession, the one after the other, then treating said twice exposed gelatine layer with water of such a temperature, that the gelatine is not dissolved even at the unexposed spots but is only caused to swell at said spots, and thereafter subjecting said printing form to the action of a ferric chloride solution.

8. A process for the photomechanical manufacture of printing forms for intaglio printing by means of a doctor which comprises covering a metallic body used as the basis for the printing form with a layer of gelatine of the trade of such a kind which only will swell on being treated with warm water without dissolving and which is rendered light sensitive by chromatizing, exposing said sensitive layer twice, under a diapositive of a continuous half-tone image and under a photogravure screen in any succession, the one after the other, then treating said twice exposed gelatine layer with water of such a temperature, that the gelatine is not dissolved even at the unexposed spots but is only caused to swell at said spots, dissolved dyes being added during this treatment, then removing said dyes again from the unexposed spots of said gelatine layer by an after-treatment with water, and thereafter bringing an etching means on said treated gelatine layer, said etching means penetrating the previously swelled parts of said gelatine layer and etching the parts of said metallic body beneath said swelled gelatine parts.

9. A process for the photomechanical manufacture of printing forms for intaglio printing by means of a doctor which comprises covering a metallic body used as the basis for the printing form with a layer of gelatine of the trade of such a kind which only will swell on being treated with warm water without dissolving and which is rendered light sensitive by chromatizing, exposing said sensitive layer twice, under a diapositive of a continuous half-tone image and under a photogravure screen in any succession, the one after the other, then treating said twice exposed gelatine layer with water of such a temperature, that the gelatine is not dissolved even at the unexposed spots but is only caused to swell at said spots, dissolved dyes and a tanning agent being added during this treatment, then removing said dyes again from the unexposed spots of said gelatine layer by an after-treatment with water, and thereafter bringing an etching means on said treated gelatine layer, said etching means penetrating the previously swelled parts of said gelatine layer and etching the parts of said metallic body beneath said swelled gelatine parts.

10. A process for the photomechanical manufacture of printing forms for intaglio printing by means of a doctor which comprises covering a metallic body used as the basis for the printing form with a layer of gelatine of the trade of such a kind which only will swell on being treated with warm water without dissolving and which is rendered light-sensitive by chromatizing, exposing said sensitive layer twice, under a diapositive of a continuous half-tone image and under a photogravure screen in any succession, the one after the other, the exposure for copying the photogravure screen being made for a longer period than that independently made for copy-

ing the continuous half-tone image and for such a time, that those parts of the sensitive layer, the surface of which is directly met by the light during the copying of the photogravure screen, are hardened with certainty down to the base of said sensitive layer, then treating said twice exposed gelatine layer with water of such a tem-

perature, that the gelatine is not dissolved even at unexposed spots, but is only caused to swell at said spots, and thereafter subjecting said printing form to the action of an etching means.

JOSEF GÖRIG.